

Feb. 25, 1941.

V. K. ZWORYKIN ET AL

2,233,276

SECONDARY ELECTRON EMISSIVE ELECTRODE

Filed March 25, 1938

2 Sheets-Sheet 1



Fig. 1



Fig. 2

Inventors  
VLADIMIR K. ZWORYKIN  
HUMBOLDT W. LEVERENZ & JOHN E. RUEDY  
By

Attorney

Feb. 25, 1941.

V. K. ZWORYKIN ET AL

2,233,276

SECONDARY ELECTRON EMISSIVE ELECTRODE

Filed March 25, 1938

2 Sheets-Sheet 2



Fig. 3.



Fig. 4.



Fig. 5.

Inventors  
VLADIMIR K. ZWORYKIN  
HUMBOLDT W. LEVERENZ & JOHN ERUEDY  
By

Attorney

## UNITED STATES PATENT OFFICE

2,233,276

## SECONDARY ELECTRON EMISSIVE ELECTRODE

Vladimir K. Zworykin, Philadelphia, Pa., and  
Humboldt W. Leverenz, Collingswood, and John  
E. Ruedy, Merchantville, N. J., assignors to  
Radio Corporation of America, a corporation of  
Delaware

Application March 25, 1938, Serial No. 197,994

7 Claims. (Cl. 250—174)

Our invention relates to secondary electron emission devices, and more specifically to a secondary electron emission device in which the secondarily emissive electrode may be formed by a compound or alloy of metallic elements. The alloy is further characterized by the fact that no activation is required to increase the secondary-electron emissibility of the electrode surface.

Secondary electron emissive devices have been known to those skilled in the art. These prior devices have included secondary emissive surfaces which require expensive and careful preparation. The stability of these surfaces, particularly at high temperatures, has been very poor. Furthermore, it has been necessary to prepare these surfaces in a vacuum, and it has been difficult to activate such surfaces for the more complicated mechanical structures such as electron multipliers.

The secondary emissive surfaces of the prior art devices have generally included a silver or silver-plated electrode. After cleaning, the electrode is mounted within a suitable envelope. The envelope is evacuated to  $1 \times 10^{-2}$  mm. of mercury and then heated and evacuated to a pressure of the order of  $1 \times 10^{-5}$  mm. of mercury. After evacuation, oxygen is introduced into the envelope and the pressure maintained at approximately 1 mm. of mercury. The silver surface of the electrode is oxidized by applying a potential of the order of 500 volts which effects a glow discharge. After the oxidation has been completed, any residual oxygen is exhausted and thereafter caesium is distilled into the envelope. The caesium combines with the silver oxide to form a suitable surface which is fixed by baking the envelope at approximately 210° C. During the baking, excessive caesium is exhausted from the envelope, which is thereafter sealed at a pressure of approximately  $1 \times 10^{-5}$  mm. of mercury. While such surfaces show an electron multiplication factor of the order of 5 to 7 at 200 volts, the devices are, as pointed out above, unstable and are not entirely suited to applications of high power with the resulting high electrode temperatures.

There have been other attempts to produce secondary emissive surfaces without employing alkali metals, but such attempts require that the emissive surfaces be formed within a vacuum and, as far as we have been able to ascertain, were not very stable at high temperatures. One of the primary purposes of our invention is to find means for producing a secondary emissive electrode which can be prepared in air, han-

dled as an ordinary metal for the preparation of electrodes, and from which high secondary emission may be obtained without any special activation within a vacuum. Another object of our invention is to form compounds or alloys of elements which in themselves do not show a high secondary emissive property but which, in combination, show satisfactory emission of secondary electrons. A still further object of our invention is to form an alloy or intermetallic compound of two or more elements which separately have low emissive characteristics, but which have a ratio of primary to secondary electron emission of the order of 5 to 7 at 200 volts and higher at higher voltages, and which are stable.

Our invention will be described by referring to the accompanying drawings, in which

Figure 1 is a chart illustrating the prior art method of forming a secondarily emissive electrode;

Figure 2 is a chart indicating the method of forming a secondarily emissive electrode in accordance with our invention;

Figure 3 is a graph showing the emissive properties of elements and their compounds made in accordance with our invention;

Figure 4 is an illustration of a secondarily emissive device; and

Figure 5 is a temperature-composition curve of the elements gold and magnesium.

Referring to Fig. 1, it will be observed that eleven successive steps are required to form a caesium-silver oxide secondary electron emissive surface. In comparison, reference is made to Fig. 2 in which, by way of example, an alloy is formed of the elements copper and magnesium. After the alloy has been formed, it is rolled into sheets from which electrodes of the desired size and shape may be stamped and formed. These electrodes, after cleaning, are mounted within an envelope such as shown in Fig. 4. The envelope with the electrodes mounted therein is heated for about one hour at 400° C. to 450° C. It is then evacuated to approximately  $1 \times 10^{-5}$  mm. of mercury and sealed. Without activation or further preparation, we have found that the alloy electrode will show a suitable ratio of primary to secondary emission and, further, that the device will be relatively stable at ordinary operating temperatures.

Referring to Fig. 3, it will be noted that the element silver has a secondary emission ratio, i. e., the ratio of primary electrons striking the element to the number of secondary electrons emitted by such impact, of the order of unity.

It will also be seen that the element magnesium has a secondary emission ratio which is of the order of two. It is difficult to explain why the compounding or the alloying of these elements should have a higher ratio than either of the elements themselves. While our invention is not to be limited to a theory which explains this anomalous situation, we believe that the increased secondary emission of the compound of the elements may be explained as follows:

When two or more elements are compounded or brought together in an alloy, the compound or the alloy does not follow the ordinary rule of chemical mixtures. The characteristics of the alloy depend not only on the proportions but also on the treatment which may result in many different molecular arrangements. Some of the different molecular arrangements of a compound or alloy which results from this treatment have been clearly illustrated by means of electron defraction and X-ray analysis. We therefore believe that the arrangement of the molecules of the compound of copper and magnesium readily lends itself to a surface which liberates secondary electrons at relatively low primary electron velocities. By way of example, we have found that good secondary emissive material may be made of alloys of magnesium with copper, silver or gold, the percentage of magnesium to the base metal element being equal to or less than the amount contained in a thermo-dynamically stable intermetallic compound of the elements. By the term "thermo-dynamically stable" is meant stability of the electrode under baking and operating conditions in a vacuum. By the term "compound" is meant a union or mixture of elements in which the elements are represented in true atomic proportions; e. g., gold Au and magnesium Mg form the following compounds: AuMg, AuMg<sub>2</sub> and AuMg<sub>3</sub>, as indicated by the maximum point or points in the temperature-composition diagram of Fig. 5.

By way of example, we have found that a fraction of one percent to the order of sixteen percent, by weight, of magnesium may be combined with copper to form a suitable alloy. By way of further examples, the following proportions may be used: of the order of 84 parts copper to 16 parts magnesium; of the order 80 parts silver to 20 parts magnesium; of the order of 70 parts gold to 30 parts magnesium; or 70 to 99.9 parts base metal to 30 to 1 parts magnesium—all by weight. Such an alloy can be readily rolled to the desired thickness and a stamping made of the desired shape to form suitable electrodes. These electrodes, after being introduced into a vacuum as described in connection with Fig. 2, will give from 4 to 6 and higher secondary electron ratios at 200 volts and upwards at higher potentials, in accordance with the curve of Fig. 3. We have found that such electrodes have surfaces which, when first subjected to electron bombardment, show a decrease in secondary emission. The surface eventually stabilizes with a comparatively high gain and thereafter remains stable at temperatures up to 600° C.

The foregoing example is not to be considered a limitation. We have made other secondary emissive electrodes of suitable emission ratio by alloying magnesium and gold, and magnesium and silver, in amounts equal to or less than the thermo-dynamically stable intermetallic compounds. It should also be understood that our use of the word "alloys" includes intermetallic compounds of the elements. The use of two ele-

ments in the specifically mentioned compounds does not exclude the use of a plurality of elements; for example, silver-copper-magnesium alloy. The final criterion of a suitable electrode is that it should be stable at high operating temperatures and preferably require no activation; therefore, we prefer to use alloys of elements which are thermo-dynamically stable at operating temperatures above the envelope baking temperature and which should have suitably high ratios of electron emission. Detailed descriptions of secondary electron emitters or multipliers will be found in the copending application Serial No. 92,563, filed July 25, 1936, by Vladimir K. Zworykin and Louis Malter.

We claim:

1. A secondary electron emissive electrode including in combination a base metal element and magnesium united in a ratio of at least two parts base metal to one part magnesium by weight and forming an alloy thermodynamically stable at operating temperatures approaching 600° C. during electron bombardment, and having a ratio of secondary electron emission to primary electron applied during bombardment of at least four.

2. A secondary electron emissive electrode formed by a compound of the elements copper and magnesium in the ratio of the order of 84 parts copper and 16 parts magnesium by weight, and having a molecular structure which exhibits thermodynamic stability at operating temperatures approaching 600° C. and a capacity to emit secondary electrons during bombardment by primary electrons.

3. A secondary electron emissive electrode formed by a compound of the elements silver and magnesium in the ratio of the order of 80 parts silver and 20 parts magnesium by weight, and having a molecular structure which exhibits thermodynamic stability at operating temperatures approaching 600° C. and a capacity to emit secondary electrons during bombardment by primary electrons.

4. A secondary electron emissive electrode formed by a compound of the elements gold and magnesium in the ratio of the order of 70 parts gold and 30 parts magnesium by weight.

5. The method of making a secondary emissive electrode from a base metal and magnesium which comprises alloying said base metal and said magnesium, forming an electrode of said alloy, cleaning said electrode, placing said electrode within an envelope, heating said envelope to approximately 450° C., and evacuating said envelope.

6. The method of making a secondary emissive electrode from base metal and magnesium which comprises alloying said base metal and said magnesium, forming an electrode of said alloy, cleaning said electrode, placing said electrode within an envelope, heating said envelope at temperatures from substantially 400° to 450° C. and until said secondary emission becomes stabilized, and evacuating said envelope.

7. The method of making a secondary emissive electrode from a base metal and magnesium which comprises alloying said base metal and said magnesium, forming an electrode of said alloy, cleaning said electrode, placing said electrode within an envelope, heating said envelope to approximately 400° C. to 450° C. for about one hour, and evacuating said envelope.

VLADIMIR K. ZWORYKIN.  
HUMBOLDT W. LEVERENZ.  
JOHN E. RUEDY.